

Patented Sept. 21, 1926.

1,600,736

# UNITED STATES PATENT OFFICE.

REUBEN F. PUNNETT, OF GREECE, NEW YORK, ASSIGNOR TO EASTMAN KODAK COMPANY, OF ROCHESTER, NEW YORK, A CORPORATION OF NEW YORK.

## ART OF LIGHT-SENSITIVE PHOTOGRAPHIC MATERIALS.

No Drawing.

Application filed June 6, 1924. Serial No. 718,409.

This invention relates to the art of photographic materials.

One object of the invention is to provide photographic sensitizing materials capable of greatly increasing the light sensitiveness of photographic emulsions especially of the developing-out type, even when incorporated therein in very small amounts. Another object is to provide such materials in concentrated and sufficiently purified condition so that they will not harmfully dilute the substances in which they are mixed. A still further object is to provide a process for obtaining said material in said desirable condition.

Another object of the invention is to provide photographic emulsions such as developing-out emulsions, having new and improved properties because of the use or presence therein of my independent sensitizing material. Still another object of my invention is to provide a process in which my said sensitizing material is used to improve photographic emulsions, especially developing-out emulsions as regards light sensitiveness, by which term I include their ability to give the earliest visible impression or image with the minimum exposure or their ability to give density after a given exposure or both, the usual photographic fluid treatments being used in preparing such impression or image.

A further object of the invention is to provide a colloid product, such as treated gelatin, the usefulness of which for forming light sensitive photographic emulsions, notably developing-out ones, is increased and controlled by my said sensitizing material incorporated therewith. Another object of the invention is to provide a corresponding process for making said intermediate colloid product.

Other objects are,—to increase the sensitiveness of photographic emulsions, particularly developing-out emulsions, while wholly or partially dispensing with expensive or long and uncertain so-called ripening methods; to enable the use of a type of gelatin having desirable physical qualities in making such a photographic emulsion of greater light sensitiveness than that normally obtainable with said gelatin; to obtain more stable emulsions through the purity of the ingredients; to increase the light sensitiveness of photographic emulsions, particularly

developing-out ones, the grain characteristics of which have already been determined; to increase the general light sensitiveness of such photographic emulsions throughout the spectral ranges to which they are normally sensitive; to make such photographic emulsions of standard light sensitive characteristics with gelatins which normally do not produce emulsions having such characteristics; to make, as intermediates in the manufacture of photographic emulsions, gelatins of standard light sensitiveness giving power out of gelatins which do not normally have the power of giving such standard sensitiveness to emulsions, such as developing-out ones made from them. Further objects will hereinafter appear.

I have found a photographic sensitizing material, very small amounts of which greatly increase the light sensitiveness of photographic emulsions, such as those of the developing-out gelatino-silver-halide type, for example. This material I have found out how to obtain in concentrated forms, so that when incorporated in such emulsions or gelatins for such emulsions, it produces its sensitivity-increasing action without harmfully diluting said emulsions or gelatins, or impairing the physical properties of them. In other words, the use of my sensitizing material furnishes a safe, practical, and largely independent way of controlling the properties of emulsions in addition to the expedients hitherto available.

While my invention is of wide utility in this art, it is especially useful in connection with gelatino-silver-halide emulsions, such, for example, as developing-out emulsions employed on negative or positive films, plates, papers, etc. The ammonia or alkaline type of such emulsions responds especially readily to my sensitizer. I shall therefore describe an illustrative embodiment of my invention in connection with such emulsions; but it will be understood that my invention is not restricted to this example except as indicated in the claims.

The first operation in practising my invention is the preparation of the sensitizing material. Being of biochemical origin, it is preferably concentrated, or separated from the organic tissues, or bulky products from such tissues, with which it is associated. For example, it originates in the tissues that yield gelatins and is carried into

the latter during their manufacture. Such gelatins especially those prepared for photographic use, are, therefore, useful sources from which my sensitizing material may be derived. Not all gelatins contain it to the same extent. To test whether any particular kind or available batch of gelatin will be a sufficiently fruitful source of sensitizer, a small sample of it can be extracted by the 10 method hereinafter described and the extract added to an emulsion, such as the one hereinafter disclosed. If the sample sensitizer causes a good increase in light sensitiveness of the emulsion, then the kind of 15 gelatin or whole batch of it can be extracted. This extraction of a sample and trial in a known emulsion provides a ready test of the raw material; but in the absence of test, practically any gelatin which can be used 20 in making sensitive emulsions can be extracted. Many gelatins, which cause bad fog when emulsions are made from them, can be extracted by my method, thus obtaining the sensitizer from material that 25 might otherwise be of little use or even pure waste.

In carrying out the invention, water—preferably distilled—is added to the gelatin at a moderate temperature, say 85° F., for 30 instance. The amount of water is conveniently in slight excess (say 10 to 20 percent) over the amount absorbed by the gelatin to swell it at said working temperature. This is allowed to stand or soak at said temperature for several days, two or three being 35 usually sufficient. During this time evaporation should be lessened or prevented, such as by keeping the wet gelatin in a closed vessel. Harmful bacterial action can be 40 prevented by adding a small amount of phenol as a preservative. Agitation of the wet gelatin during the soaking is very desirable. Vigorous shaking of it at intervals in the vessel which contains it is one satisfactory 45 way of doing this.

At the end of the soaking period, the excess watery solution, which is often somewhat viscous, can be poured off from the gelatin. The yield is improved if some of 50 the liquid also be pressed out of the gelatin, say by centrifuging it. The liquid, which has taken up the necessary substances from the gelatin, constitutes an excellent sensitizing material. Water may, however, be 55 evaporated from it, making it still more concentrated, such evaporation being conducted during the soaking, or afterward, or both. The ultimate paste, and even the substantially dry material, reached by continued 60 drying, likewise constitute concentrated sensitizing materials. Such materials are, in general, almost colorless. There are usually some break down products of gelatin in the material whether the latter be aqueous or 65 dry; but it is substantially free from un-

hydrolyzed gelatin. The sensitizing material is, therefore, for all practical purposes, freed from the bulk of organic tissues and their bulky derivatives, such as gelatin, with which it was initially associated. Stat- 70 ed in another way, the proportion of active sensitizing bodies in the final material is larger than the proportion in the sources from which it is prepared. This makes it especially useful because it can be incorpo- 75 rated into emulsions without undesirably diluting them. In other words, it increases their sensitiveness without deteriorating their other qualities such as setting ability, melting point, viscosity, grain characteris- 80 tics, etc. It establishes a ratio of sensitizing material to silver halide which is independent of the ratio of gelatine to silver halide.

The above described soaking of the gelatin and removal of the liquid with sensitizing material may be repeated as long as sufficiently rich extracts are obtained to justify the operations. During soaking I prefer to use less than 100% excess of liquid. But instead of using only a small excess of water 90 during the soaking, a large excess may be substituted and when the resulting dilute liquid is poured off from the soaked gelatine, it may be concentrated by removal of enough water until it gives a sufficiently 95 strong sensitizing action. It withstands boiling but is preferably concentrated below boiling temperature at either atmospheric or reduced pressure. After evaporation to substantial dryness, the residue may be again 100 taken up in water with the sensitizing property still present. Investigation indicates that the aqueous solution is not a true one but is colloidal. The fact that the sensitizing property remains in the dry residue and 105 in the aqueous solution shows that the sensitizing material has a very useful stability. It is generally neither markedly alkaline nor acid although it withstands both dilute acids and alkalis and can be used with them 110 in making emulsions. I classify it as organic or biochemical in distinction from inorganic material such as ammonia, silver nitrate, etc., for example. While it keeps well, bacterial action can be prevented by a little 115 phenol.

My sensitizer may be used in many ways. Broadly, it may be incorporated in emulsions or in colloids for emulsions or both. It gives additional light sensitiveness to various kinds of emulsions having different speeds and other distinctive characteristics. While it may be added at different stages of emulsion manufacture or be mixed with emulsion ingredients, either organic or inorganic, before they are mixed into the emulsion, nevertheless it can be very conveniently mixed into the emulsion when the latter is complete, ready for coating. With the grain characteristics, such as size distribution, etc., 130

already determined, and the other physical and photographic properties of the emulsion already taken care of at this stage, I can practically independently increase its light sensitiveness without impairing said other properties by adding the concentrated and purified sensitizing material described above.

As will be understood by those skilled in the art, the proportion of sensitizing material added to the emulsions will vary according to the nature of the latter, according to the concentration of the sensitizing material and according to the amount of increase in the light sensitiveness which is desired. It can be readily adjusted by trial on samples of the emulsion. When the sensitizing material is made as above described using a 10% excess of water, a useful proportion for trial is 15 parts of 20 sensitizing solution to 1000 parts by volume of emulsion. Of course, larger proportions can be employed so long as the emulsion is not harmfully diluted.

Where different batches of emulsion fall below a required manufacturing standard for light sensitiveness, although they may be otherwise satisfactory, their sensitiveness can readily be brought up to standard by mixing in my sensitizing material, the proportion varying with amount of increase which is necessary to produce a uniform product. Emulsions having almost no practical light sensitiveness but having enough of the other qualities desired in a photographic emulsion can be made usefully light sensitive by addition of my material. Thus, my sensitizing material is useful in connection with emulsions having good initial sensitiveness and those having almost no initial sensitiveness. The increase in sensitiveness can be effected in one step by thoroughly stirring all of the sensitizing material into the flowable emulsion at one time; or it may be incorporated a little at a time in successive steps.

The following example illustrates how a light sensitive photographic emulsion may be prepared and improved by the aid of my sensitizing material. Of course, my invention is not restricted to this illustration but is applicable in the cases of the very large number of widely different emulsions in this art. The emulsion forming operations hereinafter described are along the lines of known practice,—see, for instance, "Die Photographie mit Bromsilber Gelatin" by J. M. Eder, published in Halle, Germany, in 1903 by Wilhelm Knapp as Part III. of Eder's "Ausführliches Handbuch der Photographie."

The two following solutions are made up, the parts being by weight,—

A. 900 parts of silver nitrate in 9,200 parts of water.

B. 690 parts of potassium bromide and 50 parts of potassium iodide in 6,100 parts of water along with 300 parts of gelatin.

In mixing B, the halide salts are first dissolved, the water and the gelatin then added to the salt solution. Solution B is then warmed, say to 140° F., or 150° F., for example; and the silver nitrate solution A is gradually added to it with constant stirring. It is preferable to warm solution A before adding it to B, say to 150° F., or 160° F., for instance. When solution A has been thoroughly incorporated in solution B, there are then added 43 parts of strong ammonia previously dissolved in 900 parts of water. The emulsion formed by these operations is allowed to stand for a short time, say 15 minutes to a half hour, for example. Then, 1050 parts of gelatin are dissolved in it with thorough mixing. The emulsion is next cooled, such as by keeping in a cool place, until it sets to a firm jelly. The latter is broken up, as by shredding, for instance, and thoroughly washed to remove soluble salts, such as potassium nitrate and any excess potassium halides. The water is, of course, cool enough not to melt the pieces of emulsion jelly. The washed emulsion is next remelted to 100° F., and 1050 parts of water soaked gelatin are thoroughly mixed into it, the temperature then being raised, say between 120° F., and 150° F., for instance, for a short time, say a few minutes. It is then cooled and set. It is of the ammonia or alkaline type of emulsion.

My sensitizing material may be usefully incorporated at any stage of the above described process of preparing the emulsion, even being pre-mixed with solutions A or B or with the ammonia or with the gelatin at the initial stages. It is convenient to add it to the otherwise complete melted emulsion prior to coating on supports at the final stage in the process of preparing the emulsion. For example, the emulsion is remelted and there is thoroughly mixed into it 15 parts by volume of my sensitizing material (say the aqueous preparation formed as above described by using 10% excess of water over that absorbed by the gelatine) for each 1000 parts by volume of emulsion. Since the actual sensitizing bodies are only a small part of the colloidized solids in such preparation and since such solids total as only a small proportion of said liquid preparation, it follows that the actual sensitizing bodies are very useful when added in even much less than one part per thousand of emulsion by weight, in fact often less than one part in ten thousand. It will be noted that the addition of this preparation does no substantially dilute the emulsion, being of the order of two per cent or less.

With its light sensitiveness increased by

my material, the emulsion, being melted to the desired flowability, is coated on its support, such as glass, film, paper, etc., in the well known way. It is convenient to control and check the process by coating samples of the emulsion before and after the addition of my sensitizing material, the coated specimens being tried out photographically by any well known sensitometric test, or even by comparative camera exposures on the same subject. Of course, the usual precautions are observed during the emulsion making and coating process, such as the use of non-actinic or "safe" light, cleanliness of vessels and air, etc.

The different gelatins sold for photographic emulsion making may be used in the example given above, hard ones being very useful. The temperatures given are, of course, adjusted if the particular gelatin employed has physical properties, such as melting and setting points, which deviate considerably from the usual ones, such adjustment being a matter of routine control.

Instead, however, of using gelatins which give emulsions of useful but lower sensitiveness even before the addition of my sensitizing material, an almost inert gelatin may be employed—one which forms an emulsion which produces a developable image only after impractically long exposures, and then does not yield an image of desirable density. A gelatin which forms such a nearly inert emulsion may be prepared in the way described under the heading "Preparation of ash-free gelatin," on pages 1858 and 1859 of the "Journal of the American Chemical Society," September, 1922, Volume XLIV, No. 9, being part of an article by Sheppard, Sweet, and Benedict on "Elasticity of purified gelatin jellies as a function of hydrogen-ion concentration." Emulsions of impractically low light sensitiveness made by the above described process from such prepared gelatin, are transformed by my sensitizing material into emulsions which give developable images of excellent density after usefully brief exposures. I have, for example, been able to increase the light sensitiveness of such low sensitive emulsions over twenty times, the exposures for a given subject being cut to less than one twentieth of the original one and the image density being made excellent by a corresponding gain. Increases of the same general order of magnitude are made when my sensitizing material is added in similar proportions to emulsions which are made from normal photographic gelatins or mixtures of such normal gelatins with said almost inert gelatin, and already have useful but lower initial sensitiveness. Different percentages of sensitizer produce correspondingly different increases. The increases in developing-out emulsions appear

upon the usual developing operations. Customary pyro or metol-hydrochinon alkaline developers are as good as any for example.

For testing the power of sensitizing material, and almost inert emulsion made, as above described, from said prepared gelatine is also very useful. Fifteen parts by volume of the sensitizing liquid can be added to 1000 parts of such emulsion and the mixture coated and tested photographically in comparison with a parallel sample of the unsensitized emulsion. While the addition of sensitizing material as a liquid is most convenient, the residue obtained from evaporating off the water from said liquid can be added directly to the emulsion. In addition to having increased sensitiveness, emulsions containing my sensitizing material have improved stability or keeping qualities because of the purification of said material.

My sensitizing material may be incorporated into gelatin with which photographic emulsions are to be made. This "strengthened" gelatin then constitutes a valuable "intermediate" in emulsion manufacture. For example, the gelatin can be melted and 15 parts by volume of my above described aqueous sensitizing material can be thoroughly mixed into 1000 parts of gelatin. Emulsions, particularly developing-out ones made from the mixture have increased light sensitiveness as compared with those made from corresponding unstrengthened gelatin. The proportion of sensitizing material is, of course, adjusted to give the desired control of the sensitiveness of emulsions made from the gelatin, the total sensitizing material in the "strengthened" gelatin being thus brought above normal. It is especially effective when used in making emulsions having, at least slight alkalinity.

My sensitizing material acts as a so-called "chemical" sensitizer instead of an "optical" sensitizer. In other words, it increases the "general" sensitiveness of developing-out photographic emulsions in which it is incorporated; that is, to light of substantially the same wave lengths as those to which the emulsion is sensitive before my material is added; instead of merely increasing sensitiveness to light of wave lengths the same or nearly the same as those absorbed by it. It has practically no coloring properties, unlike dyes. The general sensitiveness is increased; that is, throughout the normal spectral range of the emulsion instead of at only those points corresponding to the strong spectral absorption of dye sensitizing material. My material is effective in increasing the general sensitiveness of orthochromatic, panchromatic, X-ray, and all special emulsions, as well as the ordinary or non-color-sensitized ones. It is prefer-

ably added separately or independently of the sensitizing dye generally, but not necessarily before any dye. It is especially effective in emulsions of the ammonia or alkaline type.

In the example given above the steps of treating with ammonia and warming of the emulsion just before its final setting improve the photographic properties of the emulsion; especially when the latter is made from hard gelatins. While one or both of them may be omitted I prefer to use both, in other words, my sensitizing material can act by itself to increase the light sensitivity; but ripening steps are preferably employed. The effect of either or both of such steps, is to help increase the light sensitivity of the emulsions and thus give a stronger initial sensitized condition which is multiplied or increased by using my sensitizing material. When using the ash-free gelatin mentioned above, they are quite readily dispensed with; but if retained in making very sensitive emulsions, they can be shortened and made more certain in effect by reason of the use of my powerful sensitizing material. I consider the material to be concentrated when it gives a useful effect without harmfully diluting the emulsion. It does not act as a photographic developer.

I have described gelatin emulsions because at the present time they are the ones which have the widest practical use, especially the developing-out ones. Moreover, they form the best medium for testing my sensitizing materials, the characteristic action of such materials on such emulsions being one of the best identifying criteria of such sensitizing materials. Other organic colloids and mixtures of them with each other or with gelatin, where their nature admits such mixtures, may be used in making light sensitive emulsions which can be improved by adding my sensitizing material. Albumens, agar, agar, gums, such as gum arabic, cellulosic derivatives such as collodion, are instances. While I have disclosed the use of my sensitizing material in connection with such sensitive substances as silver bromide and silver iodide, other light sensitive substances can be employed, such as silver chloride, alone or mixed with one or more of the others.

Having thus described my invention, what I claim as new and desire to secure by Letters Patent is:

1. A substantially colorless organic photographic sensitizing material derived from animal tissues, said material having the property of increasing the light sensitivity of photographic gelatino-silver-halide emulsions and being in a concentrated form substantially free from said tissues and from bulky products thereof.

2. A biochemical sensitizing material occurring in nature with gelatin and having

the property of increasing the light sensitivity of photographic gelatino-silver-halide emulsions of the alkaline type and being in concentrated form substantially free from its associated gelatin.

3. A biochemical sensitizing material derived from animal sources which acts to increase the general light sensitivity of gelatino-silver-halide emulsions of the alkaline type, when it is incorporated therein, without acting to alter the grain size characteristics thereof, said material being in concentrated form substantially free from its normally associated bulgy unhydrolyzed diluents.

4. A concentrated, purified, substantially colorless biochemical sensitizing material, which is capable, even in the absence of dyes, of increasing the light sensitivity of gelatino-silver-halide emulsions without interfering with the grain characteristics thereof, said material being substantially free from normally associated unhydrolyzed gelatin.

5. A sensitizing material from biochemical sources carried in a liquid which is harmless when mixed in light sensitive emulsions, said material having the property of increasing the light sensitivity of gelatino-silver-halide emulsions, in which it is incorporated, even in the absence of dye and inorganic sensitizers, said material having, per unit volume, greater sensitizing power than said sources.

6. A biochemical material derived from the same sources as photographic gelatin and possessing the light sensitizing principle of photographic gelatin in concentrated form substantially free from the bulk of its normally associated gelatin.

7. A light sensitive emulsion comprising a colloid, particles of photographic sensitive salts suspended therein, and an independent organic sensitizing material different from said colloid upon which at least part of the general light sensitivity of the emulsion depends.

8. A photographic developing-out gelatino-silver-halide emulsion of relatively high light sensitivity comprising a mixture of the constituents of a gelatino-silver-halide emulsion of lower light sensitivity and an independent biochemical sensitizing material upon which depends the difference between said lower and said high light sensitivity.

9. A photographic gelatino-silver-halide emulsion of the alkaline type comprising a mixture of gelatin, silver halide particles, and a biochemical sensitizing material, substantially free from its normally associated bulky impurities, which increases the light sensitivity of said emulsion.

10. A photographic gelatino-silver-halide emulsion comprising a suspension in gelatin

- of silver halide particles, and an independent biochemical sensitizing extract upon which at least part of the light sensitiveness of said emulsion depends, the volume of said extract being less than the order of 2 per cent of the total volume of the emulsion.
11. A photographic gelatino-silver-halide emulsion of relatively high light sensitiveness substantially free from dye sensitizers, comprising a mixture of the constituents of a gelatino-silver-halide emulsion, having determined grain size characteristics and lower light sensitiveness, and independent biochemical sensitizing material upon which depends the difference between said lower and said high light sensitiveness while said grain size characteristics remain substantially constant.
12. A photographic gelatino-silver-halide emulsion of the alkaline type comprising a suspension in gelatin of silver halide particles and an independent biochemical sensitizing material, the percentage of light sensitiveness due to said material being greater than the percentage of the total volume taken up by said material.
13. A photographic gelatino-silver-halide emulsion comprising a suspension in gelatin of silver halide particles and an independent biochemical sensitizing material, the proportion of the light sensitiveness of said emulsion due to said material being of the order of magnitude of 95 per cent, while the volume of the material is of the order of magnitude of 2 per cent of the volume of the emulsion.
14. A photographic gelatino-silver-halide emulsion comprising the constituents of a gelatino-silver-halide emulsion of a lower light sensitiveness of the order of one-twentieth of the light sensitiveness of the first named emulsion and an independent biochemical sensitizing extract upon which the greater light sensitiveness of the first named emulsion depends, said sensitizing extract being substantially free from effect upon the non-photographic qualities of said emulsions.
15. A photographic gelatino-silver-halide emulsion substantially free from sensitizing dye comprising a mixture of gelatin, silver halide particles, and an independent organic sensitizing material upon which at least part of the light sensitiveness of said emulsion depends, said material being substantially free from effect upon the non-photographic qualities of said emulsion.
16. A photographic gelatino-silver-halide emulsion comprising gelatin, silver halide particles suspended therein, and an independent biochemical sensitizing extract upon which at least part of the light sensitiveness of said emulsion depends, the physical properties, of said emulsion which correspond to the physical properties of said gelatin being substantially unaltered by said sensitizing extract.
17. A photographic gelatino-silver-halide emulsion having characteristics of manufacturing standard comprising the constituents of a gelatino-silver-halide emulsion of substandard light sensitiveness but otherwise of standard characteristics and an independent concentrated biochemical sensitizing material upon which the difference between said substandard and standard light sensitiveness depends, the other characteristics being substantially independent of said sensitizing material.
18. A photographic gelatino-silver-halide emulsion comprising a mixture of gelatin, silver halide particles, and an organic sensitizing material upon which at least part of the light sensitiveness of said emulsion depends irrespective of dye sensitizers, said material being substantially free from bulky colloids.
19. A photographic gelatino-silver-halide emulsion having light sensitiveness over a definite spectral range and having definite grain size characteristics, said emulsion comprising the constituents of a gelatino-silver-halide emulsion having substantially the same definite grain size characteristics but having a relatively lower light sensitiveness over said spectral range and a sensitizing material upon which depends the difference in light sensitiveness between the first named emulsion and said second named emulsion over said spectral range, the grain size characteristics being substantially independent of said sensitizing material.
20. A photographic colloid-silver-halide emulsion comprising a colloid, silver-halide particles suspended therein and a biochemical sensitizing material different from said colloid upon which the general light sensitiveness of said emulsion depends, the ratio of said material to said silver halide being substantially independent of the ratio of said colloid to said silver-halide.
21. A photographic gelatino-silver-halide emulsion comprising gelatin, silver halide particles suspended therein and a sensitizing material upon which a large part of the light sensitiveness of said emulsion depends independently of dyes, the ratio of gelatin to silver-halide being substantially unaffected by said material.
22. In the process of preparing a photographic emulsion, incorporating therein a sensitizing material derived from animal tissues but in concentrated form substantially free from said tissues and from bulky products thereof, said material increasing the light sensitiveness of said emulsion.
23. In the process of preparing a photographic gelatino-sensitive-silver salt emulsion of the alkaline type, incorporating therein a biochemical sensitizing material in

concentrated form substantially free from gelatin to increase the light sensitiveness of said emulsion.

24. In the process of preparing a photographic colloid-sensitive-silver-salt emulsion, incorporating therein a light sensitizing material which occurs in nature in gelatin sources, said material being substantially free from its associated bulky organic material and acting to increase the light sensitiveness of said emulsion.

25. In the process of preparing a photographic biochemical colloid-sensitive-silver-salt emulsion, incorporating therein a sensitizing extract different from said colloid and obtained from biochemical sources, the sensitizing power of said extract, per unit volume, being greater than that of said sources, to increase the light sensitiveness of said emulsion.

26. In the process of preparing a photographic colloid-sensitive-silver-salt emulsion, incorporating therein independently of any dye sensitizers an organic sensitizing material in concentrated form substantially free from bulky diluents, said material increasing the general light sensitiveness of said emulsion.

27. In the process of preparing a photographic colloid-sensitive-silver-salt emulsion, incorporating therein separately from dyes a biochemical sensitizing material in concentrated form substantially free from non-volatile diluents, said material increasing the general light sensitiveness of said emulsion without acting to increase the size of the grain thereof.

28. In the process of preparing a photographic developing-out gelatino-silver-halide emulsion of the alkaline type incorporating therein an organic sensitizing material in concentrated form substantially free from unhydrolyzed gelatin, said material increasing the general light sensitiveness of said emulsion.

29. In the process of preparing a photographic gelatino-silver-halide emulsion incorporating therein a sensitizing material from biochemical sources, said material having greater sensitizing power, per unit volume, than that of said sources, said material increasing the light sensitiveness of said emulsion without increasing the grain size thereof.

30. In the process of preparing a photographic gelatino-silver-halide emulsion of the alkaline type, incorporating therein sensitizing material which occurs in dilute form in organic sources and is concentrated to be more active, volume for volume, than said source, said material increasing the general light sensitiveness of said emulsion.

31. In the process of preparing a photographic gelatino-silver-halide emulsion, incorporating therein separate from any sensi-

tizing dye a sensitizing material in concentrated form substantially free from bulky diluents, said material increasing the general light sensitiveness of said emulsion without altering the grain-size characteristics thereof. 70

32. In the process of preparing a photographic gelatino-silver-bromide emulsion substantially free from sensitizing dyes, incorporating therein concentrated sensitizing material substantially free from unhydrolyzed gelatin, said material increasing the general light sensitiveness of said emulsion without acting to increase the grain size thereof. 75

33. In the process of preparing photographic gelatino-silver-halide emulsion, the steps of taking up a concentrated organic sensitizing material, independent of dye and inorganic sensitizers, in a liquid vehicle which can pass without harm into such emulsion, and incorporating the liquid carrying the material into the emulsion. 80

34. In the process of preparing a photographic gelatino-silver-halide emulsion, incorporating therein a concentrated organic sensitizing material, substantially free from bulky diluents, which increases the light sensitiveness of said emulsion irrespective of dyes and inorganic sensitizers. 90

35. In the process of preparing a photographic gelatino-silver-halide emulsion, incorporating therein a sensitizing extract from biochemical sources and having a higher sensitizing power per unit volume than said sources, said material increasing the light sensitiveness of said emulsion in addition to effects of dyes and inorganic sensitizers. 95

36. In the process of preparing photographic colloid-sensitive-silver-salt emulsions, incorporating therein an organic sensitizing material which greatly increases the general light sensitiveness of said emulsion even in the absence of dyes without substantially diluting the emulsion, the active sensitizing bodies in said material being less than one thousandth the weight of said emulsion. 105

37. In the process of preparing photographic gelatino-silver-halide emulsions of the alkaline type, incorporating therein organic sensitizing material which causes an increase in the light sensitiveness of said emulsion, the active bodies in said material being less than one thousandth the weight 110 of said emulsion. 115

38. In the process of manufacturing a photographic emulsion, extracting from a biochemical source a non-dyeing sensitizing material in a form substantially free from bulky associated diluents, and incorporating sufficient of said material and a different biochemical colloid in preparing said emulsion to increase the light sensitiveness of the latter. 120

39. In the process of manufacturing a photographic biochemical colloid-sensitive-silver-salt emulsion, extracting from organic tissues a sensitizing material different from 5 said colloid and in concentrated form substantially free from said tissues and bulky derivatives thereof, and incorporating sufficient of said material in preparing said emulsion to increase the light sensitiveness 10 of the latter.

40. In the process of manufacturing a photographic gelatino-silver-halide emulsion, extracting from a gelatin source a sensitizing material in concentrated form and 15 adding said material to said emulsion.

41. In the process of manufacturing a photographic biochemical colloid-sensitive-silver salt emulsion, extracting from a biochemical source a sensitizing material different from 20 said colloid in which the concentration of active sensitizing bodies is greater than in said source and incorporating sufficient of said material in preparing said emulsion to increase the light sensitiveness 25 of the latter.

42. In the process of manufacturing a photographic gelatino-silver-halide emulsion, extracting from a biochemical source a sensitizing material in concentrated form, and 30 incorporating in preparing said emulsion sufficient of said material to increase its light sensitiveness, said sensitizing material being free from effect on the grain size characteristics of said emulsion.

43. In the process of manufacturing a photographic gelatino-silver-halide emulsion, extracting from a biochemical source a sensitizing material in concentrated form and incorporating in preparing said emulsion sufficient of said material to increase its light sensitiveness irrespective of the action 40 of dyes and inorganic sensitizers.

44. In the process of manufacturing a photographic gelatino-silver-halide emulsion, extracting from a biochemical source a concentrated sensitizing material and incorporating said material in said emulsion to increase the light sensitiveness thereof, the proportion by volume of said material 50 being of the order of magnitude of two per cent.

45. In the process of manufacturing a photographic gelatino-silver-halide emulsion, extracting from a biochemical source a concentrated sensitizing material and incorporating approximately 2 per cent by volume of said material in said emulsion, the material increasing the light sensitiveness of said emulsion approximately 20 times.

46. In the process of manufacturing a photographic emulsion, extracting a biochemical non-dyeing sensitizing material away from at least part of its associated bulky impurities, by treatment with a fluid 60 vehicle, and incorporating sufficient of the

extract and a different biochemical colloid in preparing said emulsion to increase the light sensitiveness thereof.

47. In the process of manufacturing a photographic biochemical colloid-sensitive-silver-salt emulsion, treating an animal source containing sensitizing material associated with bulky diluents with a fluid into which said material spreads more rapidly than said impurities until said material is 70 concentrated in said fluid and freed from at least part of said diluents, and incorporating sufficient of the purified extract thus obtained in said emulsion to increase the 75 light sensitiveness thereof.

48. In the process of manufacturing photographic gelatino-silver-halide emulsion, treating a biochemical source containing a sensitizing material and bulky colloid diluents with a fluid into which said material spreads more rapidly than said diluents until an extract of material in said fluid is obtained separating at least part of said fluid from said extract and incorporating sufficient of said extract in said emulsion to 80 increase the light sensitiveness thereof.

49. In the process of manufacturing a photographic gelatino-silver-halide emulsion, extracting with water from a gelatin source a sensitizing material, and adding 95 sufficient of said aqueous extract to said emulsion to increase the light sensitiveness thereof.

50. In the process of manufacturing a photographic biochemical colloid-sensitive-salt emulsion of higher sensitiveness the steps of forming a biochemical colloid-sensitive-salt emulsion of relatively lower light sensitiveness, extracting from an animal source a sensitizing material, and incorporating sufficient of said material in said emulsion of lower light sensitiveness to change it into said emulsion of higher light sensitiveness.

51. In the process of manufacturing a photographic gelatino-silver-halide emulsion of relatively higher light sensitiveness the steps of forming a gelatino-silver-halide emulsion having definite grain size characteristics and lower light sensitiveness, extracting a sensitizing material from a biochemical source, and incorporating in said emulsion of lower light sensitiveness sufficient of said material to change it into said emulsion of higher light sensitiveness, said 120 grain size characteristics remaining substantially constant.

52. In the process of manufacturing a photographic biochemical colloid-sensitive-silver-salt emulsion of relatively higher light 125 sensitiveness, forming a biochemical colloid-sensitive silver-salt emulsion of lower light-sensitiveness and having a definite ratio of colloid to salt, extracting a biochemical sensitizing material from a biochemical source, 130

and adding sufficient of said sensitizing material to said emulsion of lower light sensitiveness to change it to said emulsion of higher light sensitiveness without substantially altering said ratio.

53. An intermediate free from silver salts and halid salts for use in making photographic emulsions comprising an emulsion-forming colloid and an independent biochemical sensitizing material different therefrom and incorporated therein, said material being substantially free from its normally associated bulky diluents, said intermediate having the property of forming emulsions of higher light sensitiveness than those formed under parallel conditions from said colloid without the material.

54. An intermediate for use in making photographic emulsions comprising a biochemical emulsion-forming colloid and an independent biochemical sensitizing material different from said colloid incorporated therein, said material being derived from a biochemical source but containing a higher concentration of active sensitizing bodies than said source, said intermediate having the property of forming emulsions of higher light-sensitiveness than those formed under parallel conditions from said colloid without the material.

55. An intermediate for forming photographic gelatino-silver-halide emulsions comprising a mixture of gelatin and an independent sensitizing material from a gelatin source, said material being substantially free from its normally associated gelatin, and said intermediate having the property of forming gelatino-silver-halide emulsions of greater general light sensitiveness than those formed under parallel conditions from said first named gelatin without said material.

56. An intermediate for forming photographic gelatino-silver-halide emulsions, comprising a mixture of gelatin and an independent biochemical sensitizing material in concentrated form, said intermediate having the property of forming gelatino-silver-halide emulsions of higher light-sensitiveness but substantially the same grain size characteristics as those formed under parallel conditions from said gelatin without said material.

57. An intermediate for use in making photographic emulsions comprising an emulsion-forming colloid and an independent sensitizing material without dye sensitizing action, said intermediate having the property of forming emulsions of higher light sensitiveness than those formed under parallel conditions from said colloid without said material.

58. An intermediate for forming photographic gelatino-silver-halide emulsions, comprising a mixture of gelatin and an in-

dependent sensitizing material in concentrated form, said intermediate having the property of forming gelatino-silver-halide emulsions of higher light sensitiveness, irrespective of the action of dyes and inorganic sensitizers, than those formed under parallel conditions from said gelatin without said material.

59. In the process of preparing an intermediate for the manufacture of photographic emulsions, the step of incorporating in an emulsion forming colloid a sensitizing material derived from an organic source but in concentrated form substantially free from said tissues and from bulky products thereof and capable of increasing the light sensitiveness of said emulsions before silver salts or halid salts are incorporated therein.

60. In the process of preparing an intermediate for the manufacture of photographic emulsions the step of incorporating in a biochemical emulsion-forming colloid an independent biochemical sensitizing material different from said colloid derived from a biochemical source but having a higher concentration of active sensitizing bodies than said source, and having the property of increasing the light sensitiveness of said emulsions.

61. In the process of preparing an intermediate for the manufacture of photographic gelatino-silver-halide emulsions the step of incorporating in gelatin an independent sensitizing material from a gelatin source but substantially free from its normally associated gelatin and having the property of increasing the light sensitiveness of said emulsions.

62. In the process of preparing an intermediate for the manufacture of photographic gelatino-silver-halide emulsions the step of incorporating in gelatin an independent concentrated biochemical sensitizing material which increases the light sensitiveness of said emulsions without affecting the grain size characteristics thereof.

63. In the process of preparing an intermediate for the manufacture of gelatino-silver-halide emulsions, the step of incorporating in gelatin an independent sensitizing material which increases the light sensitiveness of said emulsions irrespective of the action of dyes and inorganic sensitizers.

64. In the process of manufacturing an intermediate for use in making photographic emulsions, extracting from a biochemical source a sensitizing material in a form substantially free from bulky associated diluents, and incorporating said material in a photographic emulsion-forming colloid prior to the incorporation of silver salts or halid salts therein.

Signed at Rochester, New York this 4th day of June 1924.

REUBEN F. PUNNETT.